

Nov. 7, 1939.

T. W. FRECH

2,179,288

METHOD OF COATING LUMINESCENT TUBES

Filed Aug. 24, 1938



Inventor:  
Theodore W. Frech,  
by Harry E. Dunham  
His Attorney.

## UNITED STATES PATENT OFFICE

2,179,288

METHOD OF COATING LUMINESCENT  
TUBESTheodore W. Frech, Cleveland Heights, Ohio, as-  
signor to General Electric Company, a corpo-  
ration of New York

Application August 24, 1938, Serial No. 226,566

2 Claims. (Cl. 91—70)

My invention relates to the manufacture of vitreous articles having a coating of luminescent material thereon, and more particularly to a method of applying such luminescent material 5 to the inner walls of glass tubing.

Certain types of electric discharge devices, such as fluorescent lamps, have a coating of fluorescent material on the inner wall of the lamp envelope which material fluoresces or emits light when 10 excited by the rays emitted by the discharge in the device. It is well recognized that, in order to produce a lamp of maximum efficiency, the coating of fluorescent material must be of uniform thickness throughout. Various methods have 15 heretofore been proposed for applying the fluorescent coating. For example, the most common way is to mix the fluorescent material with a suitable binder which is then sprayed over the surface to be coated. Needless to say, with ordinary spray- 20 ing methods it is extremely difficult to secure a coating of uniform thickness. Other methods such as painting or the like have also been found incapable of producing a uniform coating.

One object of my invention is to provide an 25 improved method for applying a uniform coating of luminescent material to the walls of glass articles.

Another object of my invention is to provide an improved method for applying a uniform coating 30 of fluorescent material to the inner wall of a fluorescent lamp envelope.

Further objects and advantages of my invention will appear from the following description and from the accompanying drawing which is a 35 front elevation, partly in section, of the apparatus I employ in the practice of my invention.

Referring to Fig. 1, the bulb or envelope 10 to be coated is placed in the coating apparatus shown in the drawing. This apparatus comprises 40 a bottle or flask 11, preferably of spherical shape and formed with three parallel-extending neck or outlet portions, consisting of a central neck 12 and two diametrically opposite side neck portions 13 and 14. The flask 11 is firmly mounted on and 45 secured to a suitable base member 15 by means of a clamping ring 16 and tie straps (not shown) extending from said clamping ring. As shown, the flask is mounted on the base 15 so that the neck portions 12, 13 and 14 extend upwardly. The 50 said neck portions 12, 13 and 14 are provided with suitable rubber stoppers 17, 18 and 19 respectively. Extending through the stopper 17 into the body portion of the flask 11 is a propeller shaft 20 provided at its inner end with a suitable propeller 21 or other type of agitator. The

propeller shaft 20 is journaled in a combination bearing and stuffing box 22 extending through stopper 17 and secured thereto by a nut 23. The outer end of the propeller shaft 20 is coupled to the shaft 24 of a small electric motor 5 25 by means of a suitable coupling member 26. The motor 25 is secured by a mounting strap 27 to a support column or standard 28 extending upwardly from the base 15. The motor 25, together with the propeller shaft 20 coupled thereto, functions as an agitating device or mixer for a batch of coating material 29 with which the flask 11 is filled.

A pressure-supply tube 30, preferably of glass, extends through the stopper 18 into the flask 11. The said tube 30 is connected by a hose 31 to a suitable source of compressed air or gas, preferably carbon dioxide. The tube 30 is also provided with a finger valve consisting of a short length of hose 32 the free end of which is open 20 to the atmosphere. The valve 32, when open, affords free escape of the compressed air or gas entering the pressure-supply tube 30 through the hose 31.

Mounted on the stopper 19 and extending 25 therethrough down into the flask 11 is a feed tube 33. This feed tube extends to a point adjacent the bottom of the flask so that the open end of the tube will be submerged in the reservoir of coating material 29 even though the said 30 coating material, due to the using up of the same, recedes to a relatively low level. The upper portion of the stopper 19 is formed with an enlarged portion 35 having a recessed seat 36 adapted to receive the open end of the tube or bulb 10 to be 35 coated. The stoppers 17, 18 and 19 snugly fit in the corresponding flask neck portions 12, 13 and 14 so as to form a hermetic joint therebetween. Likewise, the joints or fits between the propeller shaft 20 and stopper 17, and between 40 tubes 30, 33 and stoppers 18 and 19 respectively, are also made hermetic. Thus, when the pinch tube or valve 32 is closed, the compressed air or gas entering the flask 11 through tube 30 cannot escape and so forces the coating material 29, 45 which is in a liquid state, up through the feed tube 33 into the tube or lamp bulb 10 to be coated. The elements which extend into the flask 11 and which come in contact with the coating material 29 are preferably made of stainless steel 50 so as not to become rusted; otherwise contamination of the coating material 29 might result.

The coating material 29 I employ to produce the fluorescent coating on the lamp bulb 10 consists of a mixture of binder and fluorescent ma- 55

aterial which is preferably made as follows: a binder is first prepared by dissolving 2350 grams of nitrocellulose solution in 14,900 cc. of amyl acetate. The viscosity of the resulting mixture should be between 40 to 42 seconds as measured in a Dupont #7 cup at 28° C. To 900 cc. of the above binder is added 600 grams of fluorescent material previously ground to pass a 200 mesh silk bolting cloth. This mixture is then stirred for approximately one hour in a ball mill so as to acquire a uniform consistency, whereupon 950 cc., approximately, of amyl acetate and 350 cc. of the previously mentioned binder is added and the mixture further stirred in a ball mill for approximately fifteen minutes. The mixture is then strained through a 150 mesh nickel screen and then an additional quantity of amyl acetate is added to give the proper consistency, i. e., that consistency which will give the desired thickness of coating on the lamp envelope 10 when applied by the method according to my invention.

To coat a tubular open-ended lamp bulb or tube 10 with fluorescent material by the method comprising my invention, the tube is positioned vertically on the rubber stopper 10 with the open end of the tube firmly seated in the recessed seat 36 provided therefor. The valve 32 is then closed by pinching the same, whereupon the pressure of the CO<sub>2</sub> gas entering the flask 11 through the hose 31 and pressure-supply tube 30 forces the coating material 29 up through the feed tube 33 into the lamp bulb 10. When the level of the rising coating material reaches the top of the bulb 10, the pressure is released by opening the valve 32 so that the coating material flows back into the flask 11. A deposit of coating material accordingly remains on the inner bulb walls. The coating material 29, during its application to the lamp bulb 10, is continuously agitated by rotation of the propeller 21 of the agitating device.

Following the above initial application of the coating material 29, the lamp bulb 10 is removed from the coating apparatus and placed vertically under a gentle stream of air, preferably at a pressure of approximately 14 to 15 lbs. per square inch, until the deposit of coating material is thoroughly dried. The vertical disposition of the tubular bulb allows the excess of coating material to drip off. When dried, the lamp bulb is again placed in the coating apparatus and recoated, the bulb, however, in this second coating application, being inverted from the position occupied during the first coating application. By so inverting the bulb, an extremely uniform coating is obtained. After this second coating application, the lamp bulb is again placed in the drying apparatus and the coating material air dried as described above.

To burn off the binder, the coated bulb 10, following the final drying, is fired while in a horizontal position for approximately 11 minutes in

an open-type oven at a temperature of approximately 460° C., the lamp bulb being moved through the oven in such a manner, and the gas oven burners being so adjusted as to gradually raise the temperature of the lamp bulb to the required firing temperature and then to gradually lower the bulb temperature to that of the room. As a result, no cooling strains are created in the glass lamp bulb or tube 10.

A tube or envelope prepared in accordance with the above coating method has been found to possess extremely uniform thickness of fluorescent material, and it will be obvious that various changes and modifications may be made in the described procedure without departing from the spirit and scope of the invention.

What I claim as new and desire to secure by Letters Patent of the United States is:

1. The method of applying a coating of powdered luminescent material to the inner wall of a glass tube having both ends open which comprises mounting said tube in a vertical position, flowing upwardly into said tube from the lower end thereof a coating solution containing a finely divided luminescent material in suspension, withdrawing said coating solution from said tube to thereby form a primary deposit of the solution on the inner wall of said tube, drying said primary deposit of coating solution while said tube is still in said vertical position, inverting said tube and again flowing therewith in the same manner as before the said coating solution, withdrawing said coating solution from said tube to thereby form a secondary deposit of the solution on the inner wall of said tube, and drying said secondary deposit of said coating solution while said tube is still in said inverted position.

2. The method of applying a coating of powdered luminescent material to the inner wall of a glass tube having both ends open which comprises mounting said tube in a vertical position, flowing upwardly into said tube from the lower end thereof a coating solution containing a finely divided luminescent material in suspension in a volatilizable binder, withdrawing said coating solution from said tube to thereby form a primary deposit of the solution on the inner wall of said tube, drying said primary deposit of coating solution while said tube is still in said vertical position, inverting said tube and again flowing therewith in the same manner as before the said coating solution, withdrawing said coating solution from said tube to thereby form a secondary deposit of the solution on the inner wall of said tube, drying said secondary deposit of said coating solution while said tube is still in said inverted position, and heating said tube sufficiently to volatilize the binder in the coating solution.

THEODORE W. FRECH. 60